

## UNITED STATES PATENT OFFICE

2,359,107

## COPPER-OXIDE RECTIFIERS

Carl C. Hein, Forest Hills, Pa., assignor to Westinghouse Electric & Manufacturing Company, East Pittsburgh, Pa., a corporation of Pennsylvania

No Drawing. Application September 27, 1940,  
Serial No. 358,699

4 Claims. (Cl. 175—366)

My invention relates to contact rectifiers and in particular to the methods of making electrical contacts to the operating surface-areas of such rectifiers.

One object of my invention is to provide a method for making electrical contact to surfaces of contact rectifiers in such a way that the electrical resistance of the contact will not be altered substantially by exposure to moisture and humid atmospheres.

Another object of my invention is to provide an improved method for making contact to the oxide surface of copper-oxide rectifiers.

Still another object of my invention is to provide an intermediate layer between the oxidized surface of a copper-oxide rectifier and a sprayed metal terminal area adapted to conduct current satisfactorily to the rectifier.

Other objects of my invention will become apparent upon reading the following specification.

A well known form of electrical rectifier employs an oxidized disk of metallic copper as is described in Grondahl Patent 1,640,335, assigned to the Union Switch & Signal Company, Swissvale, Pennsylvania. In such rectifiers, it is necessary to provide some arrangement for conducting current readily into the oxidized surface on the copper, such contacts being made in accordance with the description in the Grondahl patent by coating the copper oxide surface with powdered graphite and pressing a lead washer into firm contact thereon. In the process of factory production of such rectifiers the graphite has been applied in the form of a preparation having the trade name "Aquadag," manufactured by the Acheson Colloids Corporation, Port Huron, Michigan. While satisfactory for most purposes, it has been found that when rectifiers coated with Aquadag have been employed in places where they were exposed to steam or other vapors, or even in damp and humid places such as garages and basements, the electrical contact to the oxide surface apparently undergoes gradual deterioration due to some alteration in the physical or chemical condition of the graphite coating. While I do not wish my invention to be limited by any theory, I see reason to believe that the difficulty arises from some sort of attack on the graphite coating by moisture.

I have discovered that such difficulties with the graphite coating may be eliminated if it is applied in the form of a mixture comprising substantially 5 to 15% of graphite in a solvent of a high flash point naptha or the like. The percentage constituency depends upon the type of

use. For spraying, a larger amount of solvent is employed than for painting on as in the case of Aquadag. For example, the graphite product described in Bartell United States Patent 2,117,879 assigned to Acheson Colloids Corporation, New York, N. Y., made up to contain from 7.5 to 10% of solids by weight may be used for spraying.

Since the method of forming the oxidized copper disk is no part of my present invention, it will not be described in detail here; but detailed descriptions of the method of oxidizing and preparing the copper disk will be found in Conrad Patent 2,117,020, Hein Patent 2,170,200 and a detailed description of the application of the metal layer deposited upon the graphite (in this case Schoop-sprayed tin) will be found in the Aumann Patent 1,801,831.

An alternative method of applying the graphite is to employ a suspension of colloidal graphite in carbon tetrachloride in place of the mixture of graphite with high flash point naptha already described. However, the carbon tetrachloride suspension has proved less satisfactory as a factory process than has the naptha suspension described above.

Tests comparing the performance of rectifiers formed by the above described process with those in which Aquadag is used as the coating agent have clearly shown a great superiority for the former. Thus after four days in a humid atmosphere, ten rectifier plates of copper measuring  $4\frac{1}{8}'' \times 12'' \times .050''$  which employ the Aquadag treatment show an average increase of approximately 90% in resistance in the highly-conductive direction at  $12\frac{1}{2}$  ampere load, while ten exactly similar plates in the making of which the naptha solvent graphite was used averaged an increase of only about 1% in the same period.

Furthermore, the deviations in forward resistance from the average were far greater among the rectifiers coated with Aquadag than it was between the rectifiers coated with the naptha suspension graphite; the range of variation among the Aquadag rectifiers at the end of the above-mentioned four day tests was of the order of 130% of the original resistance, while the range of resistance in the naptha solvent rectifiers was only about 14% of the initial resistance. The greater constancy, and greater uniformity of forward resistance resulting from the substitution of naptha solvent graphite coats for Aquadag coats is thus evident.

While I have described one embodiment of my invention in accordance with the patent stat-

utes, its broad principles are capable of other applications which will be self-evident to those skilled in the art. Broadly speaking, I believe my contribution to the rectifier art here described to lie in the removal from the liquid in which colloidal graphite particles are suspended to form a coating mixture of hygroscopic and harmful chemical constituents. I also believe it to be evident to those skilled in the art that the method which I have developed for forming protective coatings may be applied to other contact rectifiers than the copper oxide, and in general to the production of electrical contact coatings on substances generally.

I claim as my invention:

1. The method of producing an electrical contact surface for copper oxide rectifiers which comprises applying to the oxidized surface a coating of colloidal graphite suspended in high flash-point naptha, freeing the coating of the naptha, and covering the outer surface of the coating with a metal layer. 20

5 2. The method of producing an electrical contact surface for copper oxide rectifiers which comprises applying to the oxidized surface a coating of colloidal graphite suspended in high flash-point naptha, freeing the coating of the naptha, and Schoop-spraying the outer surface of the coating with tin.

10 3. The method of forming an electrical contact to a conductor body which comprises coating the body with colloidal graphite suspended in a high flashpoint naptha solvent and freeing the coating of the solvent, and covering at least a portion of the coating with a layer of metal.

15 4. A rectifier comprising metallic copper having a portion of its surface oxidized and coated with a layer of colloidal graphite applied while suspended in a high flashpoint naptha solvent, and covered with an outer layer of metal.

CARL C. HEIN.